

Dec. 18, 1934.

W. C. VAN GEEL ET AL

1,985,118

DRY RECTIFIER

Filed Jan. 22, 1931



Inventors:  
Willem Christian van Geel,  
Jan Hendrik de Boer  
and Hendrik Bramens,

by E. F. Wiedenroth  
Atty.

## UNITED STATES PATENT OFFICE

1,985,118

## DRY RECTIFIER

Willem Christiaan van Geel, Jan Hendrik de Boer, and Hendrik Emmens, Eindhoven, Netherlands, assignors to N. V. Philips' Gloeilampenfabrieken, Eindhoven, Netherlands

Application January 22, 1931, Serial No. 510,580  
In the Netherlands March 8, 1930

7 Claims. (Cl. 175—366)

The invention relates to dry rectifiers.

Such a rectifier commonly comprises two plates, preferably of conducting material, which are placed the one on the other and between which is provided an intermediate layer of a third material.

According to the invention, the cathode of the rectifier consists, at least in part, of a metal of the first sub-group of the fourth principal group 10 of the periodic system.

It has been found that with these metals (titanium, zirconium, hafnium and thorium) a highly satisfactory rectifying effect can be obtained.

15 The cathode consisting of one of these metals is preferably coated with a layer consisting of one or more compounds of this metal. Use is preferably made of a film consisting of one or more oxides of the metal constituting the cathode.

20 It has been found that owing to the extreme permanency of the oxides of these metals the rectifiers thus produced have an almost unlimited life.

25 For the anode of said rectifiers, in which the cathode consists of a metal of the first sub-group of the fourth principal group, use should preferably be made of a compound containing as negative constituent one of the elements of the halogen group, the oxygen group or the nitrogen group or of a mixture of such compounds. For this purpose these substances while being in a powdery state, may be compressed to form plates.

30 It is often advantageous to add to the material of the anode a certain quantity of one or more of the free elements of the said groups.

35 Very favorable results have been obtained with an anode consisting of cuprous sulfide to which may be added free sulphur, and with an anode of copper iodide which may have added to it free iodine. An anode consisting of phosphor has also proved to give excellent results.

40 The metal compounds may be formed from the material of the electrode itself. This may be effected either electrolytically or chemically.

45 On heating, for example, a zirconium plate in an atmosphere of nitrogen to a temperature of 700 to 800 degrees, nitride is formed. When heating a zirconium plate in oxygen, zirconia is produced. By heating in the presence of air, a film is produced which consists of a mixture of zirconia and zirconium nitride, said film having a very satisfactory rectifying effect.

50 It is evident that for producing the rectifying layer the metal may also be dipped into chemicals.

For obtaining a surface layer on titanium, thorium or hafnium one may proceed in an analogous manner.

5 For obtaining a superficial layer by electrolysis, one may utilize, for example for the oxidation of zirconium, the electrolytes phosphoric acid, sulfuric acid, lye or ammonium borate. As the one electrode a zirconium plate is placed in the bath whereas for the other electrode use may be made of a rod of platinum, carbon or of another material which cannot be attacked. The thickness of the layer may be concluded upon by the colour which the plate assumes during oxidation. With zirconium a satisfactory thickness of the oxide layer is obtained, for example, 10 by electrolytically oxidizing until the surface of the zirconium plate has taken a yellowish green colour.

15 With the metals titanium and hafnium one may proceed in a similar manner. For thorium, 20 however, this method has proved to be less suitable so that in this case use should preferably be made of chemical means.

25 As above noted, it is advantageous to utilize for the anode cuprous sulfide to which may be added some free sulphur. If, for example, the cells are built up from a zirconium plate coated with an oxide layer and a cuprous sulfide plate one obtains a rectifier which has a very satisfactory characteristic and which appears to be 30 almost independent from temperature influences.

35 Of other materials which also give satisfactory results when they are used as anode with a cathode of a metal of the first sub-group of the fourth principal group, copper iodide to which may be added some free iodine, has already been mentioned.

40 Lead sulfide, molybdenum sulfide, tungsten sulfide, iron sulfide, iron hammer scale may also enter into consideration, more particularly if it is desired to obtain a rectifier with a slight internal resistance. In order to obtain a higher internal resistance, use may be made of an anode of manganese oxide, silver chloride with free iodine, lead dioxide and cadmium oxide. 45 The anode material may consequently be chosen in accordance with the tensions to be applied and with the current intensity to be obtained.

45 The accompanying drawing represents schematically a dry rectifier adapted to rectify a two-phase alternating current and composed of some of the above described rectifier cells.

50 The plates *a* which are coated with an oxide layer *b* consist, for example, of zirconium and constitute the cathodes. The plates *c* consist for 55

example of pressed copper iodide with free iodine. Owing to the fact that at the points where an oxide layer is present the current passes only in the direction from *c* to *a*, it will be evident that 5 in the circuit-arrangement shown full-wave rectification of the alternating current is obtained, with which during each half-cycle two elements in series are traversed.

10 The above-described rectifiers may be utilized for all purposes for which rectifiers have been utilized up to the present. In view of the manner in which the rectifier is to be utilized, it is possible to choose a suitable combination for the material of the electrodes.

15 Thus, for example a rectifier destined for a low tension and a large current intensity and whose cells consist of the combination of zirconium provided with an oxide layer and cuprous sulfide, will be particularly suitable for charging 20 accumulators, for exciting magnets and similar purposes.

25 With a rectifier of high resistance for small current intensities the cathode may consist, for example, of titanium, coated with an oxide film and the anode of manganese oxide or, again, the cathode may consist of zirconium with an oxide film and the anode of a mixture of silver chloride and free iodine. Such rectifiers may be employed, for example, in plate-tension supply 30 units.

35 What we claim is:

1. A dry rectifier having a cathode and an anode, said cathode being formed substantially of one of the metals of the first sub-group of the 40 fourth principal group of the periodic system, and a layer of oxide of the cathode metal coating said cathode, the anode comprising a metal compound which contains as its negative component one of the elements of the oxygen-group.

45 2. A dry rectifier having a cathode and an anode, said cathode being formed substantially of one of the metals of the first sub-group of the fourth principal group of the periodic system, and a layer of oxide of the cathode metal coating said cathode, the anode comprising a

5 metal compound which contains as its negative component one of the elements of the oxygen-group to which has been added a certain quantity of at least one of the free elements of the oxygen-group.

10 3. A dry rectifier having a cathode and an anode, said cathode being formed substantially of one of the metals of the first sub-group of the fourth principal group of the periodic system, a layer of oxide of the cathode metal coating said cathode, the anode comprising cuprous sulfide.

15 4. A dry rectifier having a cathode and an anode, said cathode being formed substantially of one of the metals of the first sub-group of the fourth principal group of the periodic system, a layer of oxide of the cathode metal coating said cathode, the anode comprising cuprous sulfide to which free sulphur has been added.

20 5. A dry rectifier having a cathode and an anode, said cathode being formed substantially of one of the metals of the first sub-group of the fourth principal group of the periodic system, a layer of oxide of the cathode metal coating said cathode, the anode comprising a compound which contains as its negative component 25 at least one of the elements selected from the group comprising the halogen-group, the oxygen-group, and the nitrogen-group.

30 6. A dry rectifier having a cathode and an anode, said cathode being formed substantially of one of the metals of the first sub-group of the fourth principal group of the periodic system, said anode comprising copper iodide.

35 7. A dry rectifier having a cathode and an anode, said cathode being formed substantially of one of the metals of the first sub-group of the fourth principal group of the periodic system, said anode comprising copper iodide to which 40 free iodine has been added.

45 WILLEM CHRISTIAAN VAN GEEL.  
JAN HENDRIK DE BOER.  
HENDRIK EMMENS.